

April 21, 1925.

**1,534,322**

W. HOOPES ET AL

# ELECTROLYTIC CELL AND METHOD OF LINING THE SAME

Filed Dec. 21, 1922



Inventors  
WILLIAM HOOPES  
JUNIUS D. EDWARDS  
BASIL T. HORSFIELD  
By their Attorneys  
Cooper, Kerr & Dunham

## UNITED STATES PATENT OFFICE.

WILLIAM HOOPES, OF PITTSBURGH, JUNIUS D. EDWARDS, OF OAKMONT, PENNSYLVANIA, AND BASIL T. HORSFIELD, OF BADIN, NORTH CAROLINA, ASSIGNORS TO ALUMINUM COMPANY OF AMERICA, OF PITTSBURGH, PENNSYLVANIA, A CORPORATION OF PENNSYLVANIA.

## ELECTROLYTIC CELL AND METHOD OF LINING THE SAME

Application filed December 21, 1922. Serial No. 608,289.

*To all whom it may concern:*

Be it known that we, WILLIAM HOOPES, JUNIUS D. EDWARDS, and BASIL T. HORSFIELD, all citizens of the United States of America, the said WILLIAM HOOPES residing at Pittsburgh, in the county of Allegheny and State of Pennsylvania, the said JUNIUS D. EDWARDS residing at Oakmont, in the county of Allegheny and State of Pennsylvania, and the said BASIL T. HORSFIELD residing at Badin, in the county of Stanly and State of North Carolina, have invented certain new and useful Improvements in Electrolytic Cells and Methods of Lining the Same, of which the following is a full, clear, and exact description.

This invention relates to electrolytic refining of metals, more particularly to the cell or pot in which the refining process is carried on. In the copending applications of William Hoopes, Serial Nos. 608,287, and 608,288 both filed December 21, 1922, there are described and claimed broadly an electrolytic cell and a method of providing the same with a thermally and electrically insulating side-lining, in which a side-lining of that character is formed by freezing on the inner surface of a metal shell a molten mixture of suitable materials, preferably containing aluminum and sodium fluorides and one or more other fluorides, for example barium or calcium fluorid or both, capable (at least when present in substantial amount) of raising the freezing point of the mixture. The present invention relates to similar apparatus and methods, and its chief object, briefly stated, is to provide a cell or pot having a lining, especially a side-lining, possessing in a high degree the properties of thermal and electrical insulation and of resistance to fusion. To this and other ends the invention consists in the novel features of apparatus and method hereinafter described.

The method herein described and claimed is applicable to a variety of electrolytic cells and to other containers in which a lining of the character indicated is necessary or desirable. For electrolytic refining of aluminum a cell of the general type described in the aforesaid applications of William Hoopes is particularly advantageous, and

such a cell is illustrated in the accompanying drawing, in which the cell is shown in cross section.

The apparatus illustrated comprises a lower steel shell 10 of cylindrical form and an upper steel shell 11, the two constituting the lower and upper sections of the complete shell. The shell sections are secured together in any convenient manner, and are electrically separated or insulated from each other as indicated by the insulating ring or gasket 12. They are also provided with cooling means, as for example annular water jackets 13, 14, in the neighborhood of the joint between the two sections. Cooling water is supplied to the lower water jacket through a pipe 15 and inlet nipple 16 and flows in both directions to an outlet nipple 17. Thence it passes through pipe 18 and inlet nipple 19 to the upper water jacket, in which it flows in both directions to the outlet nipple 20 and thence through pipe 21 to the waste pipe 22. To prevent electrical grounding, rubber hose may be used for the pipes 15 and 21, and rubber hose may be used for the pipe 18 to prevent material flow of current from one cell section to the other. It will be understood that the water used should be sufficiently pure to be substantially non-conducting at the voltage employed in the cell. In the bottom is a layer of heat insulating material 23, and on this is a bottom lining 24 of conducting material, as for example carbon. Good electrical connection is afforded by metal collector plates 25 welded to the inside of the lower shell section and embedded in the carbon bottom. Electrical connection between the lower shell and the external circuit or source of current, not shown, may be made by means of a terminal or busbar 26 welded or bolted to the shell. The carbon bottom, which constitutes the lower electrode of the cell, is formed with a cavity or depression in its top, as indicated, and with a tapping hole 27, which may be closed by a plug 28 of suitable refractory material, as for example a dense charcoal plug. The upper electrode 100 may be of multiple form, comprising a suitable number of carbonaceous cylinders or rods 29 in the upper ends of which the copper or other metal rods 30 are secured.

Electrical connection may be made between these metal rods and the external circuit or source of current by means of a terminal or busbar 31 to which the rods are clamped or otherwise secured in any convenient and suitable manner, not shown.

On the sides of the cell is a thermally and electrically insulating lining 32, in close union with the carbon bottom 24 and extending over the joint between the shell sections to a plane well up in the upper section. In accordance with the preferred practice of our present invention for use in electrolytic refining of aluminum, this side-lining has, as an essential ingredient, alumina in corundum-like form; and is formed by freezing a crust on the sides of the cell, from a molten mixture having a composition (and containing alumina) adapted to cause selective crystallization upon the cell walls of a layer of different composition and containing a substantial amount of alumina. Preferably the mixture contains aluminum, barium and sodium fluorids.

25 The following is a convenient and effective method of forming the side lining in a cell of the type illustrated:

The upper electrodes (which for this purpose may be composed of amorphous carbon) are lowered into contact with the carbon bottom and current is sent through the cell from the upper electrodes to the lower, resulting in generation of heat at the points of contact. Powdered or granular bath mixture, preferably with a suitable amount of a high melting substance, is deposited in the cell, and after a sufficient quantity has been melted the upper electrodes are raised so that the current is compelled to pass through the fused bath. Molten metal or alloy of suitable character, heavier than the bath, is now poured into the bottom of the cell, thereby raising the bath so that the upper electrodes must be raised farther to keep their lower ends out of contact with the metal, and more bath material is supplied until the cell is filled to the desired height. The bath should, however, remain in contact with the carbon bottom-lining at the edges of the cavity therein, and if the cell is intended for use in refining aluminum the metal employed to raise the bath is preferably an aluminum alloy in composition the same as or similar to that which is to be refined in the subsequent refining operation of the cell. In the meantime water is circulated through the water jackets, and the high melting constituent in powdered or granular form is fed to the bath, preferably in amount sufficient to keep the bath saturated therewith. Under such conditions there is formed on the cooled portions of the shell sections, by selective crystallization thereon, a hard, firmly adherent crust 60 of substantial thickness, having a different

composition from that of the fused or liquid bath and containing a large amount of the high melting ingredient in coarsely crystalline form. A crust thus produced from a fluorid mixture containing alumina as the chief high melting constituent has a freezing point such that temperatures as high as 1050° C. can subsequently be used in the cell without fusing the crust, and even higher temperatures if the crust is cooled, as by means of the water jackets. Nor is the crust attacked in any substantial degree in subsequent use of the cell with a bath composed of fused fluorids; and since the alumina crystals are large they suffer but little by the solvent action of such baths, whereas in crusts formed from unsaturated mixtures the alumina is deposited in the crust in the form of extremely fine particles which are readily redissolved.

85 The mechanism of the formation of the above described side-lining crust by our improved method appears to be as follows:

Alumina becomes more soluble in cryolite baths as their temperature is raised, but if alumina be added until the bath is approximately saturated, it will be found that a small drop in temperature will cause some of the alumina to precipitate out as corundum or in corundum-like form, with which more or less bath will be mechanically associated.

In an operating cell the portion of the bath adjacent to the walls is at a temperature distinctly lower than that of the main body of the bath, so that if sufficient alumina is employed to saturate this main body the natural circulation will cause a gradual deposition of part of the alumina on the walls of the cell in the form of a thickened crust. By reason of their moderate rate of growth, the alumina crystals in this crust tend to attain a relatively considerable size, so that the crust when broken shows a coarsely crystalline structure.

110 After the crust has been built up to a suitable thickness, its formation may be arrested by reducing the alumina content of the bath. This may be done, for example, by removing part or all of the bath and replacing it with fresh bath of similar or suitable composition, but substantially free from alumina. Another and more convenient means consists in stopping the addition of alumina to the bath and electrolyzing the latter, using a carbon anode and a heavy molten alloy cathode, and thus deoxidizing the bath by electrolytic reduction of alumina. When the bath has been brought to a satisfactory condition, the cell may be put in operation, for electrolytic refining, by the method described in the aforesaid applications of William Hoopes. The crust formation can also be arrested by breaking the connection with the source of

90

95

100

105

110

115

120

125

130

current and removing the molten bath, as by dipping it out.

For aluminum refining the side-lining crust may be composed of or formed from a mixture containing alumina and aluminum fluorid and one or more alkali metal or alkaline-earth metal fluorids, as for example barium, sodium, and strontium. The presence of chlorids of the metals mentioned is 10 permissible but in general is not desirable. Calcium and magnesium fluorids are also permissible. A mixture composed of or containing, by weight, about 9 parts aluminum fluorid, 9 parts barium fluorid, and 7 parts 15 sodium fluorid, with enough alumina to saturate the mixture, has been found eminently satisfactory, and so has also (with the addition of alumina) the bath or electrolyte mixture described in a copending application of William Hoopes, Francis C. Frary, and Junius D. Edwards.

The voltage and amperage needed to fuse the mixture depend largely upon its composition and the quantity to be melted, the 25 size of the cell and the effectiveness of its heat-insulation, etc., and hence it is impossible to give definite figures which would be universally applicable. In practice the power input is regulated to produce fusion 30 of the materials and maintain them at the desired temperature. With a cell constructed as and in about the proportions indicated in the accompanying drawing, a voltage between 7 and 9 volts and a current 35 density of 800 amperes per square foot were found satisfactory for use with the fluorid and alumina mixture stated quantitatively above.

The preferred method of forming the 40 boundary crust or side-lining has been described above. It is, as already intimated, highly desirable that this crust should be made as non-conductive as possible, both electrically and thermally, since thermal 45 conductivity permits excessive loss of heat to the water jacket, thus increasing the power consumption required to maintain the operating temperature, and electrical conductivity permits current to pass from anode 50 to cathode without depositing metal on the latter, thus decreasing the current efficiency. The crust is composed of frozen materials with considerable portions of alumina in corundum-like form. These materials when 55 cold, if uncontaminated by impurities, have the desired electrically and thermally insulating properties but they become more or less electrically conductive when hot. It is important, in forming the crust, to exercise 60 care to maintain the bath, from which the crust is formed, substantially free from carbon and finely divided metal, which, if present, tend to be included in the crust and render it conductive at the time of formation. Covering the carbon bottom of the cell 65

with a layer of metal as soon as possible in order to minimize the amount of carbon exposed, aids in maintaining the bath in a carbon-free condition. Having the top part of the shell electrically neutral during the 70 crust-forming stage is also very advantageous. If this part of the shell is allowed to be negative in the stage referred to, metallic reduction products, especially sodium, tend to accumulate in the crust and render 75 it conductive. If, on the other hand, it is allowed to be positive, iron tends to dissolve and contaminate the bath, and the resultant corrosion may cause penetration of the water jacket. 80

We have described above the formation of our electrically and thermally insulating refractory side lining, in a cell which is just being started. During the operation of the cell, it is found that oxygen is introduced 85 into the bath, resulting in the formation of alumina therein, due to a number of causes; among which may be especially mentioned the cathodic production of sodium, its oxidation by the air, and the return of the resulting products to the molten bath. Unless suitable measures are taken to remove alumina from the bath electrolytically or otherwise, its concentration will gradually increase, and soon the deposition of alumina 90 upon the insulating lining, and the consequent thickening thereof, will begin. When this lining reaches an undesirable thickness, its inner surface will have become so hot, 95 due to the lessened flow of heat to the water jacket, that the concentration of alumina in equilibrium with it in the bath will be relatively high. If this crust be now broken out and removed, a new crust containing 100 alumina in corundum-like form will be 105 promptly produced from the bath and the alumina which it contains, and the concentration of the latter in the bath will be correspondingly reduced. This cycle repeats 110 itself from time to time, and thus the crust rich in alumina serves not only as an excellent insulating lining, but as a convenient means of removing excess alumina from the bath, in the method described and claimed broadly in the copending application of 115 William Hoopes and Francis C. Frary, Serial No. 608,286 filed December 21, 1922.

It is recognized that, strictly speaking, the aluminum lying floating on the bath and the layer of alloy underlying the bath, are the upper and lower electrodes, respectively, but these layers are termed herein the cathode and the anode, and hence it is deemed permissible as well as convenient to refer to the graphite cylinders and the carbon bottom-lining, or their equivalents, as the upper and lower electrodes. 120 125

It is to be understood that the invention is not limited to the apparatus and procedure herein specifically illustrated or described. 130

but can be carried out in other ways without departure from its spirit.

We claim—

1. The process of producing a refractory insulating lining for an electrolytic cell, comprising freezing from a fused bath therein a lining containing the constituents of the bath in substantially different proportions from those in the liquid and substantially more refractory than a lining having the same composition as the liquid. 70
2. The process of producing a refractory insulating lining for an electrolytic cell, comprising compounding and fusing a bath adapted for selective crystallization, upon the walls of the cell, of a lining containing the constituents of the bath in substantially different proportions from those in the liquid and substantially more refractory than a lining having the same composition as the liquid; and cooling the cell walls to cause such selective crystallization thereon. 75
3. The process of producing a refractory insulating lining for an electrolytic cell, comprising freezing from a fused bath a lining containing a high-melting bath constituent of limited solubility and forming thereby a more refractory lining than one having the same composition as the fused bath. 80
4. The process of producing a refractory insulating lining for an electrolytic cell, comprising compounding and fusing a bath adapted for selective crystallization, upon the walls of the cell, of a lining containing a high-melting constituent of limited solubility, and producing thereby upon said walls a lining more refractory than one having the same composition as the fused bath. 85
5. The method of lining an electrolytic cell for the electrolysis of fused salts which consists in establishing in the cell a fused bath otherwise suitable to act as an electrolyte in the use of the cell but charged with a refractory material desired as a constituent of said lining, and depositing from the mixture a crystalline crust containing said material on desired portions of the cell walls. 90
6. The method of lining an electrolytic cell for the electrolysis of fused salts which consists in establishing in the cell a bath of fused material suitable to act as the electrolyte, charging said bath with a material more refractory than the normal electrolyte and suitable as a constituent of said lining, and cooling portions of the said walls whereby an adherent crystalline crust containing said material is deposited thereon from said bath. 95
7. The process of producing a refractory insulating lining for an electrolytic cell, comprising freezing from a fused bath in the cell, by cooling the walls of the cell, a lining containing a high-melting material which is a constituent of the bath but which is of limited solubility therein, and producing thereby a more refractory lining than one having the same composition as the fused bath. 100
8. In the electrolytic refining of aluminum, the process of producing a refractory insulating lining for the refining cell, comprising freezing a lining upon the walls of the cell from a fused bath therein containing alumina and having a composition adapted to cause selective crystallization upon said walls of a layer rich in alumina and substantially more refractory than a layer having the same composition as the fused bath. 105
9. In the electrolytic refining of aluminum, the process of producing a refractory insulating lining for the refining cell, comprising establishing in the cell a fused fluorid bath containing alumina and having a composition adapted to selectively crystallize upon the walls of the cell a layer containing sufficient alumina to render it substantially more refractory than a lining having the same composition as the fused bath, and freezing such a layer upon the walls of the cell. 110
10. In the art of lining a cell or vessel for electrolytic refining and for other purposes, the improvement comprising freezing a coating on the interior surface of the cell out of a fused mixture containing one or more metal fluorids and alumina in amount sufficient to substantially saturate the mixture. 115
11. In the art of lining a cell or vessel for electrolytic refining and for other purposes, the improvement comprising covering the sides of a metal shell with a molten mixture containing one or more metal fluorids and alumina, and freezing from such mixture on the sides of the shell a crust or lining containing alumina in coarsely crystalline corundum-like form. 120
12. In the art of lining a cell or vessel for electrolytic refining and for other purposes, the improvement comprising freezing a coating on the interior surface of the cell out of a fused mixture containing aluminum fluorid and alumina, the latter being in amount sufficient to substantially saturate the mixture. 125
13. In the art of lining a cell or vessel for electrolytic refining and for other purposes, the improvement comprising applying to the inner surface of a metal shell a molten mixture containing about 9 parts of aluminum fluorid, 9 parts of barium fluorid, 7 parts of sodium fluorid, and alumina, and freezing from such mixture on the sides of the shell a crust or lining containing alumina in coarsely crystalline corundum-like form. 130
14. In the art of lining a cell or vessel for electrolytic refining and for other purposes, the improvement comprising fusing in the cell a mixture containing in solid form one or more metal fluorids and alumina and

passing current through the fused portion of such mixture to continue fusion of the same, and freezing from the mixture on the inside of the cell a lining containing alumina in coarsely crystalline corundum-like form.

15. In the art of lining a cell or vessel for electrolytic refining and for other purposes, the improvement comprising generating heat in the cell by electrical energy and fusing by such heat a mixture containing aluminum, barium, and sodium fluorids, and alumina, and freezing from the fused mixture on the interior surface of the cell a crust having a freezing point higher than that of the same fluorids when unsaturated with alumina.

16. In the art of lining a cell or vessel for electrolytic refining and for other purposes, the improvement comprising generating heat in the cell by electrical energy and fusing by such heat a mixture containing about 9 parts of aluminum fluorid, 9 parts of barium fluorid, and 7 parts of sodium fluorid, and alumina, and freezing from the fused mixture on the interior surface of the cell a crust or lining containing alumina in coarsely crystalline corundum-like form.

17. In the art of lining a cell or vessel for electrolytic refining and for other purposes, the improvement comprising fusing in the cell a mixture containing one or more metal fluorids and freezing on the inner surface of the cell, while supplying alumina to the fused mixture, a crust or layer containing alumina in corundum-like form.

18. In the electrolysis of a fused bath in a cell having a lining composed of bath ingredients in solid form, the steps comprising accumulating in the bath a high-melting ingredient thereof, removing more or less of the lining, and selectively crystallizing on the cell walls a solid lining composed of bath ingredients but containing said high-melting ingredient in excess.

19. In the electrolysis of a fused bath containing a high-melting ingredient of limited solubility, in a cell having a lining composed of bath ingredients in solid form, the steps

comprising removing more or less of the lining, and selectively crystallizing on the cell walls a lining of bath ingredients with said high-melting ingredient in a proportion adapted to make the lining more refractory than one having the same composition as the remaining bath.

20. In the electrolytic refining of aluminum with a fused bath containing alumina in a cell having a lining composed of bath ingredients in solid form, the steps comprising removing more or less of the lining, and selectively crystallizing thereon a lining containing alumina in higher proportion than in the liquid.

21. In the electrolysis of a fused bath in a cell having a lining composed of bath ingredients in solid form, the steps comprising removing more or less of the lining, and cooling the cell walls to selectively crystallize thereon from the bath a solid layer containing bath ingredients in substantially different proportions and substantially more refractory than a lining having the same composition as the remaining bath.

22. A cell or vessel for electrolytic refining and for other purposes, having a thermally and electrically insulating lining composed of one or more metal fluorids and alumina in coarsely crystalline corundum-like form.

23. A cell or vessel for electrolytic refining and for other purposes, comprising a metal shell having a lining composed essentially of one or more metal fluorids and alumina in coarsely crystalline corundum-like form.

24. A cell or vessel for electrolytic refining and for other purposes, comprising a metal shell having an interior side-lining composed of one or more metal fluorids and alumina in coarsely crystalline corundum-like form.

In testimony whereof we hereto affix our signatures.

WILLIAM HOOPES.  
JUNIUS D. EDWARDS.  
BASIL T. HORSFIELD.